

1

2,860,976

ANTIFOGGANTS FOR PHOTOGRAPHIC  
DEVELOPERS

Catherine M. Spath, Rochester, N. Y., assignor to Eastman Kodak Company, Rochester, N. Y., a corporation of New Jersey

No Drawing. Application August 3, 1956  
Serial No. 602,067

11 Claims. (Cl. 96—22)

This invention relates to photographic developers, and more particularly, a method of inhibiting or preventing fog during development.

It is known that when a developer acts upon an exposed emulsion layer, some of the silver halide grains which have not been exposed to light or radiation are reduced to metallic silver. This metallic silver in the unexposed portions of the emulsion results in unwanted density and this density is known as fog. Fog may be formed as a result of the chemical characteristics of the developing agent, the particular silver halide emulsion, or both. In order to produce effective results in various photographic processes, it is, accordingly, necessary to inhibit fog both in the emulsion layers and in the photographic developing solutions. While it may be important to inhibit fog as much as possible in black-and-white photography, it is even more important in reversal color processes, where the exposed emulsion layers are given a first development in a black-and-white developer, followed by reversal exposure and development in a color developer. Otherwise a proper color balance is not obtained since sufficient silver halide is not available in the appropriate areas of the emulsion layer for subsequent development with a color developer.

The unwanted density occurring as a result of the action of the black-and-white developer is particularly apparent in those portions of the emulsion layers intended to record the cyan image, i. e., where no red area, or a reduced amount of red, is present in the original subject. A similar effect occurs in the emulsion layers intended to record the magenta and yellow images.

I have now found an improved means of controlling the unwanted density resulting during black-and-white development of photographic silver halide emulsions. Silver halide emulsions which have been subjected to a first development for producing a black-and-white image, followed at some later stage by color development for producing a cyan image, and which contain a fog-inhibiting agent in the first developer as outlined below, have improved contrast and color density.

It is, accordingly, an object of my invention to provide improved developers in photographic processes. Another object is to provide a method of inhibiting the fog resulting from the action of certain black-and-white developers. Still another object is to improve the accuracy of rendition of color images, particularly in the cyan layer of multilayer photographic elements which have been differentially sensitized to record specific regions of the spectrum. Other objects will become apparent from a consideration of the following description and examples.

According to my invention, I provide improved photographic developers containing 4-carboxythiazolidines, or water-soluble salts thereof, in addition to the usual alkaline agent and black-and-white developing agent.

2

The 4-carboxythiazolidines useful in practicing my invention can advantageously be represented by the following general formula:



wherein R represents a hydrogen atom, an alkyl group (e. g., methyl, ethyl, etc.), especially a lower alkyl group, or an aryl group, such as phenyl, o-, m- and p-hydroxyphenyl, o-, m- and p-chlorophenyl, o-, m- and p-methoxyphenyl, o-, m- and p-nitrophenyl, o-, m- and p-diethylaminophenyl, etc. (e. g., a monocyclic aryl group of the benzene series) and R<sub>1</sub> represents a hydrogen atom or a cation, such as an alkali metal atom (e. g., sodium, potassium, lithium, etc.), an ammonium ion, or an organic ammonium ion, such as pyridinium (R<sub>1</sub> is hydrogen), triethyl ammonium (R<sub>1</sub> is hydrogen, etc. The term carboxyl as used herein is intended to define the COOH group as well as water-soluble derivatives thereof. If desired, the compounds of Formula I can be added to the strongly alkaline developing agents in the form of their esters which are easily hydrolyzed, such as methyl or ethyl esters, to give the desired water-soluble alkali metal salts.

The 4-carboxythiazolidines useful in practicing my invention are added to the developers commonly employed in the photographic art for producing black-and-white images. Such developers include the compounds known as polyhydroxybenzenes (e. g., hydroquinone, catechol, pyrogallol, etc.), and N-substituted aminophenols (e. g., N-methylaminophenols, N-ethylaminophenols, etc.) or mixtures of such developers. Prominent among such developing agents for the rapid development of photographic images are those comprising hydroquinone and Elon (p-N-methylaminophenol). While such developing agents and mixtures thereof give high speeds, they have the undesirable characteristic of producing density in regions of the emulsion where no exposure took place. The additives of my invention eliminate or materially reduce deposits of silver in unwanted portions of the emulsion layers.

It has been previously proposed to incorporate various 4-carboxythiazolidines in small quantities in photographic silver halide emulsions, however, these additives cause a loss in sensitivity in the emulsions in certain cases and sufficient quantity thereof does not find its way into the developing solutions to be of any material benefit. It has been unexpectedly found that addition of these 4-carboxythiazolidines to black-and-white developers has a marked beneficial effect on the characteristics of the resulting image, particularly in photographic reversal color processes.

4-carboxythiazolidines (and water-soluble salts thereof) which have been found particularly useful in practicing my invention include the following:

- (1) 4-carboxythiazolidine
- (2) 4-carboxy-2-(p-nitrophenyl)thiazolidine
- 60 (3) 4-carboxy-2-(4-hydroxy-3-methoxyphenyl)thiazolidine
- (4) 4-carboxy-2-(p-hydroxyphenyl)thiazolidine
- (5) 4-carboxy-2-(p-chlorophenyl)thiazolidine
- (6) 4-carboxy-2-(o-chlorophenyl)thiazolidine
- 65 (7) 4-carboxy-2-(m-nitrophenyl)thiazolidine
- (8) 4-carboxy-2-(o-nitrophenyl)thiazolidine
- (9) 4-carboxy-2-(p-diethylaminophenyl)thiazolidine
- (10) 4-carboxy-2-n-hexylthiazolidine

The above 4-carboxythiazolidines can be prepared according to the method described by Tegima et al. in "J. Chem. Soc. Japan," Ind. Chem. Sect., vol. 52 (1949), pages 336-8, and vol. 54 (1951), pages 648-51.

The 4-carboxythiazolidines employed in the developers of my invention can be utilized in various concentrations, depending on the particular emulsions employed and the concentration of silver halide in the emulsions and concentration of developing agents in the developers. In general, not less than 10 mg. per liter of developer of 4-carboxythiazolidine should be employed. The most advantageous concentration of 4-carboxythiazolidine compound can be determined by developing a series of test strips of silver halide emulsions wherein the concentration of the 4-carboxythiazolidine compounds is varied, as well as the concentration of developing agent (if desired). The usual addenda can be employed in the developers, such as strongly alkaline agents (e. g., sodium carbonate, potassium carbonate, sodium hydroxide, etc.), restrainers, such as potassium bromide, stain preventives, such as alkali metal sulfites, etc.

My invention is primarily directed to the development of the ordinarily employed gelatino-silver-halide developing-out emulsions, e. g., gelatino-silver-chloride, -chlorobromide, -chloroiodide, -chlorobromiodide, -bromide and -bromiodide developing-out emulsions. While the results in the following examples were obtained using gelatino-silver-bromiodide emulsions, excellent results have also been obtained using other silver halide emulsions. These emulsions can be coated in the usual manner on any suitable support, e. g., glass, cellulose nitrate film, cellulose acetate film, polyvinyl acetal resin film, paper or metal.

Photographic silver halide emulsions useful in my invention can also contain such addenda as chemical sensitizers, e. g., sulfur sensitizers (e. g., allyl thiocarbamide, thiourea, allyl isothiocyanate, cystine, etc.), various gold compounds (e. g., potassium chloroaurate, auric trichloride, etc.) (see U. S. Patents 2,540,085; 2,597,856 and 2,597,915), various azaindene compounds (such as those disclosed in U. S. Patent 2,716,062), condensation products of alkylene oxides, such as those shown in U. S. Patent 2,400,532, as well as the additives mentioned in Jones et al. U. S. application Serial No. 575,160, filed March 30, 1956.

As mentioned above, the advantages of my invention are particularly outstanding in reversal color photographic processes. This includes processes where the color couplers are incorporated in the color developers or where the color-forming compounds are incorporated in the photographic emulsions. Where the color-forming compounds are incorporated in the photographic emulsions, it is generally desirable to disperse the same in an appropriate dispersing medium, such as is shown in U. S. Patents 2,322,027 or 2,304,940. Typical color-forming compounds which can be employed in my invention include the following:

#### COUPLER

- (1) 1-hydroxy-2-[ $\delta$ -2',4'-di-tert.amylphenoxy]-n-butyl]-naphthamide (U. S. Patent 2,474,293)
- (2) 1-hydroxy-4-phenylazo-4'-(p-tert.-butylphenoxy)-2-naphthanilide (U. S. Patent 2,521,908)
- (3) 2-(2,4-di-tert.amylphenoxyacetamino)-4,6-dichloro-5-methyl phenol (U. S. Patent 2,725,291)
- (4) 2-( $\alpha$ -di-tert.amylphenoxy-n-butyrylamino)-4,6-di-chloro-t-methyl phenol
- (5) 6-{ $\alpha$ -{4-[ $\alpha$ -(2,4-di-tert.amylphenoxy)butyramido]-phenoxy}acetamido}-2,4-dichloro-3-methyl phenol
- (6) 2-[3'-(2',4"-diamylphenoxy)-acetamido]-benzamido-4-chloro-5-methyl phenol
- (7) 1-(2',4',6'-trichlorophenyl)-3-[3'-(2",4"-di-tert.amylphenoxyacetamido)-benzamido]-5-pyrazolone (U. S. Patent 2,600,788)
- (8) 1-(2',4',6'-trichlorophenyl)-3-[3'-(2",4"-di-tert.amylphenoxyacetamido)-benzamido]-4-(p-methoxyphenylazo)-5-pyrazolone

- (9) N-(4-benzoylacetaminobenzenesulfonyl)-N-( $\gamma$ -phenylpropyl)-p-toluidine (U. S. Patent 2,298,443)
- (10)  $\alpha$ -o-Methoxybenzoyl- $\alpha$ -chloro-4-[ $\alpha$ -(2,4-di-tert.amylphenoxy)-n-butyramido]-acetanilide (McCrossen U. S. application Serial No. 295,806)
- (11)  $\alpha$ -{3-[ $\alpha$ -(2,4-di-tert.amylphenoxy)acetamido]-benzoyl}-2-methoxyacetanilide
- (12) 3-benzoylacetamido-4-methoxy-2',4'-di-tert.amylphenoxy acetanilide
- (13) 4-benzylacetamido-3-methoxy-2',4'-di-tert.amylphenoxy acetanilide

The above couplers are primarily useful for use in photographic silver halide emulsions as contrasted with other couplers which are primarily useful in color developers. Couplers which are primarily useful in color developers have previously been described in a number of patents and technical articles. Spence and Carroll U. S. Patent 2,640,776, issued June 2, 1953, enumerates 20 a number of couplers useful in color developers which have been found particularly useful in my invention. Typical of such couplers for producing cyan images are:

#### COUPLER

- (14) 5-(p-aminophenoxybenzenesulfonamino)-1-naphthol
- (15) 2,4-dichloro-5-palmitylamino-1-naphthol
- (16) 8-hydroxy-1- $\alpha$ -naphthoyl-1,2,3,4-tetrahydroquinoline
- (17) 5-phenoxyacetamino-1-naphthol
- (18) 2-acetylamino-5-methylphenol
- (19) 2-{4'- $\alpha$ -(4'-tert.amylphenoxy)-n-butyrylamino}-benzoylamino}-4-chloro-5-methylphenol
- (20) 2,4-dichloro-5-(p-toluenesulfamino)-1-naphthol

Other couplers can also be advantageously employed in my invention and it is to be understood that the above lists are merely representative and are not intended to limit my invention. Couplers for producing magenta images and yellow images have also been described elsewhere, including U. S. Patent 2,640,776. These couplers can also be employed in color processes of the type herein described.

#### Example 1

**Negative development.**—A portion of a gelatino-silver-bromiodide emulsion which had been sensitized with a sulfur compound and a gold compound as mentioned above was coated on a cellulose acetate support (identified as coating 1 below). The oleyl ether of a polyethylene glycol having a molecular weight greater than 300 was added to a second portion of this emulsion at a concentration of 5 grams of the oleyl ether per mole of silver halide, and the emulsion was coated on a cellulose acetate support (identified as coating 2 below). One strip of each coating was exposed for  $\frac{1}{25}$  second to a 500-watt, 3000° K. light source on an Eastman type Ib sensitometer. The exposed coatings were then developed for three minutes in developer A having the following composition:

|                                   |       |    |      |
|-----------------------------------|-------|----|------|
| Sodium hexametaphosphate          | ----- | g  | 0.5  |
| Sodium sulfite (anhydrous)        | ----- | g  | 40.0 |
| N-methyl-p-aminophenolsulfate     | ----- | g  | 5.0  |
| Hydroquinone                      | ----- | g  | 2.0  |
| 65 Sodium carbonate (monohydrate) | ----- | g  | 25.0 |
| Potassium bromide                 | ----- | g  | 1.0  |
| Potassium iodide (0.1% solution)  | ----- | cc | 2    |
| Water to make one liter.          |       |    |      |
| (pH was 10.1 at 70° F.)           |       |    |      |

An exposed strip of each coating was developed in a composition having the same formula as developer A above, except that 0.15 g. per liter of 4-carboxy-2-(p-chlorophenyl)thiazolidine was added. This second developer is identified below as developer B. The series of

coatings was then fixed in a solution having the following composition:

Sodium thiosulfate (pentahydrate) -----g. 200  
Sodium sulfite (anhydrous) -----g. 10  
Water to make one liter.

The coatings were washed in the usual manner and dried.

**Color development.**—Two additional strips of each of the above coatings (1 and 2) were exposed and processed in developers A and B described above and washed for two minutes. These coatings were then given a reversal exposure for ten seconds (flash) with No. 2 Photofloods set at 52 inch distance. The coatings were then developed for five minutes in a developer having the following formula:

|                                                       |      |
|-------------------------------------------------------|------|
| Sulfuric acid (conc.) -----cc.                        | 0.7  |
| Hydroxylamine hydrochloride -----g.                   | 2.0  |
| Sodium hexametaphosphate -----g.                      | 0.5  |
| Sodium sulfite (anhydrous) -----g.                    | 5.0  |
| Color developer <sup>1</sup> -----g.                  | 0.55 |
| Sodium carbonate (monohydrate) -----g.                | 15.0 |
| Potassium bromide -----g.                             | 0.25 |
| 6-nitrobenzimidazole nitrate (1/2% solution) -----cc. | 4    |
| Potassium iodide (0.1% solution) -----cc.             | 2    |
| Coupler <sup>2</sup> -----g.                          | 1.2  |
| Sodium hydroxide -----g.                              | 0.3  |
| Water to make one liter.                              |      |

<sup>1</sup> 4-amino-3-methyl-N,N-diethylaniline hydrochloride.  
<sup>2</sup> 2,4-dichloro-5-(p-toluenesulfonylamo)-1-naphthol.

The coatings were washed for ten minutes and treated for two minutes in a silver bleach bath having the following composition:

|                                |     |
|--------------------------------|-----|
| Potassium ferricyanide -----g. | 100 |
| Potassium bromide -----g.      | 10  |
| Borax -----g.                  | 7.5 |
| Boric acid -----g.             | 5.0 |
| Water to make one liter.       |     |

The coatings were then treated for two minutes in a fixing bath having the composition given above, washed and dried. The speed and fog for each of the above coatings were measured after the washing following negative development, while the D-max. on the color developed strips was measured after completion of the process (i. e., after cyan development). The speed figures given below were determined according to the formula: speed equals 100 (1-log E) wherein E is the exposure in meter candle seconds required to give a density of 0.3 above fog. The results obtained were as follows:

#### NEGATIVE DEVELOPMENT

| Coating | Developer | Speed | Fog  |
|---------|-----------|-------|------|
| (1)     | A         | 115   | 0.39 |
| (1)     | B         | 112   | 0.15 |
| (2)     | A         | 121   | 0.58 |
| (2)     | B         | 115   | 0.20 |

#### COLOR DEVELOPMENT

| Coating | Developer | D-Max. |
|---------|-----------|--------|
| (1)     | A         | 2.36   |
| (1)     | B         | >4.00  |
| (2)     | A         | 3.27   |
| (2)     | B         | >4.00  |

The improvement obtained as a result of the use of the 4-carboxythiazolidine compound when measurement is made before color development and after color development is immediately apparent, both in emulsions unsensitized chemically with a polyethylene glycol derivative and with emulsions so sensitized.

#### Example 2

An ordinary photographic gelatino-silver-bromide emulsion was divided into two portions and 5 g. of the oleyl ether of polyethylene glycol per mole of silver halide was added to one portion, and these portions coated on separate cellulose acetate supports, identified (1) (unsensitized) and (2) (sensitized). The coatings were exposed and processed exactly as described in Example 1 above except that 4-carboxy-2-(m-nitrophenyl)thiazolidine was added to one of the black-and-white developers in the amount of 0.03 g. per liter of developer in place of the corresponding chloro compound employed in Example 1. The developer containing no thiazolidine compound is identified as A below, while the developer containing said compound is identified as B below. The processed coatings were then examined, as in the case of Example 1, for fog and speed after the first development and the color density (D-max.) after the color development. The results obtained were as follows:

#### NEGATIVE DEVELOPMENT

|        | Coating | Developer | Speed | Fog  |
|--------|---------|-----------|-------|------|
| 25 (1) |         | A         | 115   | 0.39 |
| (1)    |         | B         | 119   | 0.12 |
| (2)    |         | A         | 121   | 0.58 |
| (2)    |         | B         | 126   | 0.16 |

#### COLOR DEVELOPMENT

|        | Coating | Developer | D-Max. |
|--------|---------|-----------|--------|
| 30 (1) |         | A         | 2.36   |
| (1)    |         | B         | >4.00  |
| (2)    |         | A         | 3.27   |
| 35 (2) |         | B         | >4.00  |

In a manner similar to that described above, other 4-carboxythiazolidine compounds can be incorporated in black-and-white developers to give less fog. Particularly useful 4-carboxy-thiazolidine compounds include those represented by Formula I above wherein R represents an aryl group.

The photographic silver halide emulsions useful in the processes described above can be prepared according to known methods, such as those described in Hewitson and McClintock U. S. Patent 2,618,556, issued November 18, 1952. Such emulsions can be chemically sensitized according to the method described in the copending application Serial No. 550,495, filed December 1, 1955, in the name of D. E. Piper.

The color-forming developers useful in my invention have been previously described in the prior art, and my invention is not to be restricted to the use of any particular color-forming developer. The most useful of such color-forming developers are the phenylenediamines and substituted derivatives thereof. Typical of such color-forming developers are the sulfonamido substituted p-phenylenediamines disclosed in Weissberger et al. U. S. Patent 2,548,574, issued April 10, 1951, the substituted p-phenylenediamines disclosed in Weissberger et al. U. S. Patents 2,552,240-2, issued May 8, 1951, and the substituted p-phenylenediamines disclosed in Weissberger et al. U. S. Patent 2,566,271, issued August 28, 1951. Other phenylenediamine color-forming developers can be employed to like advantage in the process of my invention.

While the above examples primarily illustrate the use of photographic emulsions which have been chemically sensitized with the oleyl ether of polyethylene glycol, it is to be understood that other condensates of alkylene oxides can be advantageously employed to sensitize such emulsions. Such condensates are generally referred to as alkylene oxide polymers, the alkylene oxides generally containing from 2 to 4 carbon atoms. Such alkylene oxide polymers include polyalkylene glycols and condensation products of alkylene oxides with organic compounds

containing an active hydrogen atom, such as alcohols, amines, mercaptans, acids, amides, etc. Generally, such alkylene oxide polymers have a molecular weight of at least 300, as shown in U. S. application Serial No. 550,495, mentioned above. It is to be further understood that the emulsions employed in my invention need not be chemically sensitized, although particularly useful results have been obtained with emulsions which have been chemically sensitized with such alkylene oxide polymers.

What I claim as my invention and desire secured by Letters Patent of the United States is:

1. A photographic developer having a reduced tendency to fog photographic silver halide emulsions comprising an alkaline solution of (1) a silver halide developing agent selected from the group consisting of polyhydroxybenzenes, N-monoalkylaminophenols, and mixtures of said polyhydroxybenzenes and N-monoalkylaminophenols and at least 10 mg. per liter of solution of (2) a compound selected from the group consisting of (A) those represented by the following general formula:



wherein R represents a member selected from the group consisting of a hydrogen atom, a lower alkyl group containing from 1 to 2 carbon atoms and a monocyclic aryl group of the benzene series, and (B) a water-soluble salt of said compound.

2. A photographic developer having a reduced tendency to fog photographic silver halide emulsions comprising an alkaline solution of hydroquinone and N-methyl-p-aminophenol, and at least 10 mg. per liter of solution of a water-soluble salt of a compound selected from those represented by the following general formula:



wherein R represents a member selected from the group consisting of a hydrogen atom, a lower alkyl group and a monocyclic aryl group of the benzene series.

3. A photographic developer having a reduced tendency to fog photographic silver halide emulsions comprising an alkaline solution of a silver halide developer selected from the group consisting of polyhydroxybenzenes, N-monoalkylaminophenols and mixtures of said polyhydroxybenzenes and N-monoalkylaminophenols and at least 10 mg. per liter of solution of a water-soluble salt of a compound selected from those represented by the following general formula:



wherein R represents a monocyclic aryl group of the benzene series.

4. A photographic developer having a reduced tendency to fog photographic silver halide emulsions comprising an alkaline solution of (1) a photographic silver halide developer selected from the group consisting of hydroquinone, N-methyl-p-aminophenol and mixtures of hydroquinone (2) an N-methyl-p-aminophenol, an alkali metal sulfite and (3) at least 10 mg. per liter of solution of a water-soluble salt of a compound selected from those represented by the following general formula:



wherein R represents a monocyclic aryl group of the benzene series.

5. A photographic developer having a reduced tendency to fog photographic silver halide emulsions comprising an alkaline aqueous solution of hydroquinone, N-methyl-p-aminophenol and at least 10 mg. per liter of solution of a water soluble salt of 4-carboxy-2-(p-chlorophenyl)-thiazolidine.

6. A photographic developer having a reduced tendency to fog photographic silver halide emulsions comprising an alkaline aqueous solution of hydroquinone, N-methyl-p-aminophenol and at least 10 mg. per liter of solution of a water soluble salt of 4-carboxy-2-(m-nitrophenyl)thiazolidine.

15 7. In a complete photographic reversal color process wherein a multilayer photographic element containing a plurality of differentially sensitized photographic silver halide emulsion layers is given a first exposure, followed by development in a photographic developer for producing a black-and-white negative image and a second exposure followed by at least one additional development in a photographic developer for producing a colored image, said colored image bearing a complementary relationship to the region of the spectrum to which the photographic silver halide emulsion has been differentially sensitized, the step of developing said photographic silver halide emulsion layers after the first exposure with a black-and-white developer comprising an alkaline solution of a silver halide developing agent selected from the group consisting of polyhydroxybenzenes, N-monoalkyl-aminophenols and mixtures of polyhydroxybenzenes and N-monoalkyl-aminophenols and at least 10 mg. per liter of solution of a compound selected from the group consisting of (1) those represented by the following general formula:



40 wherein R represents a member selected from the group consisting of a hydrogen atom, a lower alkyl group containing from 1 to 2 carbon atoms and a monocyclic aryl group of the benzene series, and (2) a water-soluble salt of said compound.

45 8. In a complete photographic reversal color process wherein a multilayer photographic element containing a plurality of differentially sensitized photographic silver halide emulsion layers is given a first exposure, followed by development in a photographic developer for producing a black-and-white negative image and a second exposure followed by at least one additional development in a photographic developer for producing a colored image, said colored image bearing a complementary relationship to the region of the spectrum to which the photographic silver halide emulsion has been differentially sensitized, the step of developing said first exposed silver halide emulsion layers in a black-and-white photographic developer having a reduced tendency to fog said photographic silver halide emulsions comprising an alkaline solution of hydroquinone and N-methyl-p-aminophenol, 50 and at least 10 mg. per liter of solution of a water-soluble salt of a compound selected from those represented by the following general formula:



wherein R represents a member selected from the group consisting of a hydrogen atom, a lower alkyl group containing from 1 to 2 carbon atoms and a monocyclic aryl group of the benzene series.

9. In a complete photographic reversal color process wherein a multilayer photographic element containing a plurality of differentially sensitized photographic silver halide emulsion layers is given a first exposure, followed by development in a photographic developer for pro-

ducing a black-and-white negative image and a second exposure followed by at least one additional development in a photographic developer for producing a colored image, said colored image bearing a complementary relationship to the region of the spectrum to which the photographic silver halide emulsion has been differentially sensitized, the step of developing said first exposed silver halide emulsion layers in a black-and-white developer having a reduced tendency to fog said silver halide emulsions comprising an alkaline solution of a photographic silver halide developer selected from the group consisting of hydroquinone, N-methyl-p-aminophenol and mixtures of hydroquinone and N-methyl-p-aminophenol, an alkali metal sulfite and at least 10 mg. per liter of solution of a water-soluble salt of a compound selected from those represented by the following general formula:



wherein R represents a monocyclic aryl group of the benzene series.

10. In a complete photographic reversal color process wherein a multilayer photographic element containing a plurality of differentially sensitized photographic silver halide emulsion layers is given a first exposure, followed by development in a photographic developer for producing a black-and-white negative image and a second exposure followed by at least one additional development in a photographic developer for producing a colored image, said colored image bearing a complementary relationship to the region of the spectrum to which the photographic silver halide emulsion has been differentially sensitized, the step of developing said first exposed silver halide emulsion layers in a black-and-white photographic developer having a reduced tendency to fog said photographic silver halide emulsions comprising an aqueous solution of (1) a photographic silver halide developer selected from the group consisting of hydroquinone, N-methyl-p-aminophenol, and mixtures of hydroquinone and N-methyl-p-aminophenol, (2) sodium carbonate, (3) an alkali metal sulfite, and (4) a compound selected from those represented by the following general formula:



wherein R represents a monocyclic aryl group of the benzene series.

- 5 11. In a complete photographic reversal color process wherein a multilayer photographic element containing a plurality of differentially sensitized photographic silver halide emulsion layers, at least one of which is chemically sensitized with an alkylene oxide polymer having a molecular weight of at least 300, said alkylene oxide containing from 2 to 4 carbon atoms, is given a first exposure, followed by development in a photographic developer for producing a black-and-white negative image and at least one additional exposure followed by at least one additional development in a photographic developer for producing a colored image, said colored image having a complementary relationship to the region of the spectrum to which the photographic silver halide emulsion has been differentially sensitized, the step of developing said first exposed silver halide emulsion layer in a black-and-white photographic developer having a reduced tendency to fog said photographic silver halide emulsions, comprising an alkaline solution of a silver halide developing agent selected
- 10 20 from the group consisting of polyhydroxybenzenes, N-monoalkylaminophenols and mixtures of polyhydroxybenzenes and N-monoalkylaminophenols and at least 10 mg. per liter of solution of a water-soluble salt of a compound selected from those represented by the following general formula:



30 35 wherein R represents a member selected from the group consisting of a hydrogen atom, a lower alkyl group containing from 1 to 2 carbon atoms and a monocyclic aryl group of the benzene series.

#### References Cited in the file of this patent

#### UNITED STATES PATENTS

- 40 2,099,374 Schwarz \_\_\_\_\_ Nov. 16, 1937

#### OTHER REFERENCES

- Chem. Abstracts, 44, 1490a (1950).  
 Chem. Abstracts, 46, 2937c (1952).  
 Chem. Abstracts, 46, 10025a (1952).  
 Chem. Abstracts, 47, 1514g (1953).  
 Chem. Abstracts, 47, 6803e (1953).  
 Chem. Abstracts, 48, 11394b (1954).  
 Chem. Abstracts, 49, 15575h (1955).